

# United States Patent Office

3,266,958

Patented August 16, 1966

1

3,266,958

## HIGH ENERGY FUEL COMPOSITION CONTAINING POLYBUTADIENE AND BORANE

Jack D. Breazeale, Grand Island, Charles F. Parks, Buffalo, and Robert V. Wright, Grand Island, N.Y., as signors to Olin Mathieson Chemical Corporation  
No Drawing. Filed July 18, 1958, Ser. No. 749,559

21 Claims. (Cl. 149—19)

This invention relates to reaction products of polybutadiene rubbers and boranes.

Polybutadiene is a well known synthetic rubber material. Polybutadiene is available, for example, as the products known as "Butarez," a trade name of the Phillips Petroleum Company.

It has now been found that certain boranes can be combined with polybutadiene to form a solid material of high boron content suitable for use as a propellant fuel for rocket power plants and other jet propelled devices.

The fuels of this invention when incorporated with suitable oxidizers, such as ammonium perchlorate, potassium perchlorate, sodium perchlorate, ammonium nitrate and etc., yield solid propellants suitable for rocket power plants and other jet propelled devices. Such propellants burn with high flame speeds, have high heats of combustion and are of the high specific impulse type. Probably the single most important factor in determining the performance of a propellant charge is the specific impulse. Appreciable increases in performance will result from the use of the higher specific impulse materials. The fuels of this invention when incorporated with oxidizers are capable of being formed into a wide variety of grains, tablets and shapes all with desirable mechanical and chemical properties. Propellants produced by the methods described in this application burn uniformly without disintegration when ignited by conventional means, such as the pyrotechnic type igniter and are mechanically strong enough to withstand ordinary handling.

An important advantage of the fuels of this invention is that they are elastic and hence resist cracking by heat and thermal shock. In practical use, solid propellants for jet propelled devices may be exposed to a variety of temperature conditions. Wide variations in temperatures cause thermal expansions which may induce cracking in the propellant grains. Similarly, physical shock experienced by the propellant grains both before and during their discharge in jet propelled devices may cause fracture and cracking of the grains. Such cracked propellant grains can be extremely dangerous to the jet propelled device in that they permit the grain to burn more rapidly in the immediate vicinity of the cracked section. The uneven burning rate which results may be so great as to cause an uneven thrust by the jet engine or an explosion in the rocket power plant. It is therefore very essential that the propellant used not be subject to fracture. Compounds having a rubber-like quality are particularly desirable for use in propellant grains because they can absorb both thermal and mechanical shock without cracking or fracturing. The natural resiliency and elastic qualities of rubber-like materials make them ideal for resisting fracture. The fuel of this invention will not deteriorate when stored over a wide range of temperature conditions. It can be produced in a uniform composition, can easily be cast into grains and will not crack. In addition, the high percentage of boron which is present in the propellant composition is in a readily burnable form and results in the release of much larger quantities of energy than the corresponding composition of carbon. The fuels of this invention need not use the conventional binding agent used by many other similar compounds to cause the oxidizer and fuel to adhere. The cohesive and tacky quality of

2

the final product is sufficient to bind into a solid mass the granular oxidizing agent which is admixed with the fuel. Such mass will retain its form and elastic qualities when shaped into various configurations, and when cast into grains will adhere to the walls of the rocket case.

According to this invention, a polybutadiene is reacted with a suitable borane to produce solid materials useful as propellant fuels.

The polybutadiene rubbers suitable for use in this invention are solids or liquids. They include the known liquid and solid polymers obtained by polymerization of butadiene by various methods, e.g., sodium catalysis. The liquid products known as "Butarez" are particularly useful.

15 The physical properties of liquid polybutadiene (Butarez-15, Phillips Petroleum Company) are as follows:

| Property:                         | Value  |
|-----------------------------------|--------|
| API gravity, 60° F.               | 24.3   |
| Specific gravity, 60° F.          | 0.9083 |
| Density, 60° F., lbs./gal.        | 7.5    |
| Refractive index, $n_{20}/d$      | 1.5198 |
| Iodine number                     | 32.5   |
| Color, Gardner                    | 11     |
| Volatile material, wt. percentage | 1.0    |
| Viscosity, SFV at 100° F.         | 1500   |

The liquid polymerization product of butadiene as exemplified by Butarez-15 is primarily a linear polymeric chain built by random of 1,4 and 1,2 addition during the polymerization reaction of C-4 units of the two types indicated below:



35 The polymer ordinarily contains 55 to 65 percent of 1,2 addition units and approximately 0.8 double bonds per C-4 unit. Ultraviolet scanning techniques indicate the presence of conjugate structures of the naphthalenic type possibly derived from cyclization. Some cross-linking of the polymer chain is also evident.

40 The repeating formula of emulsion polymerized polybutadiene (a solid) is  $-(\text{CH}_2\text{CH}=\text{CHCH}_2)_n$ . The physical properties are as follows:

| Property:                      | Value           |
|--------------------------------|-----------------|
| Density at 25° C. (G. per cc.) | 0.89            |
| Refractive index at 25° C.     | 1.5148          |
| Average mol. wt.               | 100,000-200,000 |
| Dilute solution viscosity      | 1.93            |
| $[\eta]$ Intrinsic viscosity   | 2.08            |

45 A liquid emulsion polymerized polybutadiene can also be used.

| Property:                 | Typical value |
|---------------------------|---------------|
| Ash, percent              | 0.02          |
| Moisture, percent         | 0.102         |
| Dilute solution viscosity | 0.18          |
| Viscosity SFV at 210° F.  | 496           |

50 60 The polybutadienes useful in this invention have an average molecular weight range of about 1,000 to about 3,000,000.

65 The boranes suitable for use in this invention are decaborane and lower alkyl decaboranes in which the alkyl group contains from 1 to 5 carbon atoms, or mixtures of decaborane and alkyl decaboranes. Such alkyl decaboranes include, for example, monomethyldecaborane, dimethyldecaborane, monoethyldecaborane, diethyldecaborane, triethyldecaborane and monoisopropyl decaborane. Mixtures of alkyl decaboranes can be used. Alkyl decaboranes can be prepared by reacting decaborane and an alkyl halide in the presence of an alkylation catalyst

as described in pending application Serial No. 497,407, filed March 28, 1955, now Pat. No. 2,999,117, of Altwicker et al. and in pending application Serial No. 540,141, filed October 12, 1955, of Altwicker et al. now Pat. No. 3,109,030 wherein ferric chloride is used as the catalyst. Monoethyldecaborane can be also prepared by the reaction of decaborane and ethylene as described in pending application Serial No. 514,121, filed June 8, 1955, of Stange et al. Also, alkylated decaboranes such as monoethyldecaborane and diethyldecaborane can be prepared by reacting a mono-olefin hydrocarbon with a mixture of decaborane and an aluminum halide as described in pending application Serial No. 557,634, filed January 6, 1956, of Neff et al. now Pat. No. 2,987,552.

The polybutadiene is generally reacted with the borane at temperatures ranging from about 20 to 300° C. and pressures from about atmospheric to 1,000 p.s.i. The time of reaction varies from about 0.25 to 50 hours or more, depending on the temperature and pressure employed. The borane is used in an amount of about 0.05 to 10 parts per part of polybutadiene, and preferably from 0.5 to 3.5 parts of the borane per part of polybutadiene. A solvent for the polybutadiene and inert to the reaction, e.g., methylcyclohexane, can be used if desired. The solvent can be used in amounts of from 0.001 to 100 parts of solvent per part of polybutadiene. The liquid polybutadiene can be reacted with the decaborane or alkyl decaborane with or without the use of a solvent. When solid polybutadiene is used, preferably it is dissolved in a solvent before reaction with decaborane or first plasticized, e.g., with alkyl decaborane, before reaction with decaborane.

The reaction product can be cured by carrying out the reaction under appropriate curing conditions of temperature and pressure or by first forming the reaction product and then curing it. Curing agents such as decaborane or the alkyl decaboranes can be used as well as conventional cures, applicable to polybutadiene, e.g., a sulfur cure. The curing agents can be present during the reaction or used in a later curing step after separate formation of the reaction product.

For the preparation of propellant compositions containing an oxidizer, the oxidizer can be added to the reaction mixture, including the curing agent if it is present, and the reaction and curing carried out in the presence of the oxidizer or the oxidizer can be added to the separately formed reaction product before curing or the oxidizer can be added to the separately formed and cured reaction product, e.g., by intimately admixing it into the product.

The solid materials produced by the reaction of polybutadiene and the various boranes described above are elastic or rubber-like to resinous solids of varying hardness and colors. Some are tacky. They are non-pyrophoric but burn readily on ignition. The solids contain a substantial amount of boron and with the boron admixed with or linked to the rubber molecule.

This invention will be further illustrated by reference to the following examples, wherein the polybutadienes used were those described above.

#### Example I

Solid emulsion polymerized polybutadiene (1.0 gram) dissolved in methylcyclohexane (20 grams) was placed with decaborane (1.0 gram) in a Chrome Vanadium Micro reaction vessel (American Instrument Company) of 110 cubic centimeter capacity. The autoclave was charged as above in a dry box, then sealed and placed in a rocking mechanism which permitted rocking during the heating period. The reaction mixture was maintained at temperature of 150° C. for 3 hours at a pressure of 30-35 pounds per square inch guage after which it was cooled to room temperature. The pressure of the vessel after cooling was essentially atmospheric (similar to starting pressure) indicating no gas was evolved. The product ob-

tained was then filtered and subjected to reduced pressure (1 to 2 mm. of mercury) to remove the methylcyclohexane and was then extracted with pentane (100 ml.) to remove the unreacted decaborane. After removal of the pentane by subjecting to reduced pressure for 7 hours, a brown resilient material was obtained which was found, by Parr Bomb peroxide fusion analysis, to contain 3.74 percent boron.

#### Example II

Solid emulsion polymerized polybutadiene (1.0 gram) dissolved in methylcyclohexane (20 grams) was placed with decaborane (1.0 gram) in a Chrome Vanadium Micro reaction vessel (American Instrument Company) of 110 cubic centimeters capacity. The autoclave was charged as above in a dry box then sealed and placed on a mechanism which permitted rocking during the heating period. The reaction mixture was maintained at a temperature of 250° C. for three hours, during which time the pressure in the sealed system increased from 80 to 150 pounds per square inch guage. After cooling the autoclave to room temperature, the product was removed and separated from the solvent by decantation. The product obtained was extracted with methylcyclohexane (100 ml.) to remove unreacted decaborane, and then was subjected to reduced pressure (1-2 mm. of mercury) for 7 hours to remove this solvent. A black resinous solid material was obtained which was found, by Parr Bomb peroxide fusion analysis, to contain 3.7 percent boron.

#### Example III

5 grams of sodium polymerized liquid polybutadiene (Butarez-15, Phillips Petroleum Company) was mixed with 20 cc. of methylcyclohexane and 1.0 gram of decaborane in a Chrome Vanadium Micro reaction vessel (American Instrument Company) of 110 cubic centimeter capacity. The autoclave was charged as above in a dry box, was sealed and placed on a mechanism which permitted rocking during the heating period. The reaction mixture was maintained at a temperature of 200° C. and at a pressure of 45 pounds per square inch guage for 30 minutes after which it was cooled to room temperature. The product obtained was extracted with 100 ml. of pentane to remove unreacted decaborane and then subjected to reduced pressure (1-2 millimeters of mercury) for 7 hours to remove the excess solvent. A black, sticky material was obtained which was found, by Par Bomb fusion analysis, to contain 5.63 percent boron.

#### Example IV

The preparation of the proposed fuel was started by dissolving decaborane (8.8098 g.) in diethyldecaborane (349.283 g.). This solution then was mixed with solid emulsion polymerized polybutadiene (81.110 g.) in the following manner: a trial sample of polybutadiene (4.8 g.) was placed on a small hand operated mill and to this diethyldecaborane (25 cc. or about 20.6 g.) was added from a syringe (in a dry box). The mixture was found to be too fluid to handle conveniently on this mill, so it was transferred to a Waring Blender, which was swept with nitrogen. The remainder of the diethyldecaborane, containing decaborane, and the polybutadiene were added in increments with stirring. The mixture then was poured into a sample bottle and reserved for evaluation. Qualitative examination showed the material as prepared to be almost completely soluble in benzene. Parr sodium peroxide fusion gave analysis of 42.7, 41.8 and 43.3 percent boron on the original mixture.

A sample of the original mixture (5.9 g.) is then mixed with powdered ammonium perchlorate (20.0 g.) on a small hand operated mill. The resulting compound is cured in a Carver press for 16 hours at about 55° C., to form an elastomeric material. Benzene extraction provides a product which is 81 percent gel which contains 7.7 percent boron.

## Examples V and VI

A solution of 5.0 g. of sodium-polymerized liquid polybutadiene (Butarez-15) and 2.5 g. of decaborane in 20 cc. of methylcyclohexane was transferred to an American Instrument Company 406-35B6 Micro Reaction Vessel of 110 ml. capacity. After flushing with nitrogen, the vessel was sealed, placed on the rocking mechanism and heated at 200° C. for one-half hour at a pressure of 40 to 45 p.s.i.g. The dark brown gelatinous material obtained was washed with 50 cc. of n-pentane in four batches, and then subjected to reduced pressure for 10 minutes to remove the solvent. The product obtained was shown by Parr Bomb sodium peroxide fusion to contain 16.35 percent boron. Example VI described in Table 1, was performed in a similar manner.

## Examples VII and IX

A syringe was used to add 8.9793 g. of triethyldeca-  
10 borane to 1.5005 g. of solid emulsion polymerized polybutadiene in a mortar and pestle. After mulling to produce intimate contact, the mixture was allowed to stand for about 96 hours. A portion of the tacky gum which resulted was placed in a mold in a Carver press for 16 hours at 55° C. The cured material thus obtained was found to contain 42.4 percent boron, and to have a gel content of about 0.51 percent. Examples VII and VIII described in Table 2 were performed in a similar manner.

## Examples X to XII

A 1.1131 g. portion of a mixture containing 4.7008 g. of monoethyldeca-  
20 borane and 1.9981 g. of solid emulsion polymerized polybutadiene, prepared by mulling in a mortar and pestle, was placed on a small mill. To this was added 0.0113 g. of decaborane and milling was continued until the mixture appeared homogeneous. The material thus obtained was placed in a Carver press for 16 hours at 55° C. The cured material thus obtained was found to contain 47.5 percent boron, and to have a gel content of 24 percent. Examples XI and XII described below in Table 3 were performed in a similar manner.

## Examples XIII to XV

To a 200 ml. round glass stoppered flask was added 1.0101 g. of solid emulsion polymerized polybutadiene, followed by 10.0077 g. of benzene. Then 0.0205 g. of sulfur and 0.0217 g. of Butyl Eight (a dithiocarbamate type ultra-accelerator) were added, the flask was swept with nitrogen, and 1.0694 g. of monoethyldeca-  
30 borane was added. The benzene solvent was removed under reduced pressure in about 2 hours at 30° C., leaving 2.1288 g. (100.3 percent recovery) of the fuel mixture. The material then was cured in an oven at 55° C. for 16 hours, scraped from the flask, and cut up into small pieces.

These were extracted with 100.7677 g. of benzene in a Soxhlet extractor, and then dried and weighed to determine gel content, which was found to be 48.7 percent of the fuel mixture. The boron content of this gel portion was found to be 2.4 percent. Examples XIV and XV described in Table 4 below were performed in a similar manner.

## Example XVI

10 In an 8 oz. bottle, 6.08 g. of Phillips solid emulsion polymerized polybutadiene and 45 ml. benzene were agitated gently 15 hours to form a solution. A solution of 0.015 g. triethylamine in 15 ml. benzene was added and again mixed.

15 In a nitrogen atmosphere, 8.1 g. of triethyldeca-  
borane was added, and the gray green mixtures were agitated gently 30 minutes. The benzene was removed by vacuum evaporation at room temperature for several hours.

The residue, which at this point was rubbery and elastic, was heated in a curing mold at 60° C. for 3 hours. No effort was made to exclude air during the molding.

20 The product was firm, tough, transparent and free of bubbles. It had a gel content of 27 percent, and the gel contained 2.9 percent boron. A sample sealed in an air-free glass tube (nitrogen filled) possessed almost all of its original properties at 6 months.

## Examples XVII to XX

30 4.45 g. of Phillips solid emulsion polymerized polybutadiene was dissolved in 50 ml. of benzene. A nitrogen atmosphere was maintained, and 0.0114 g. of diphenylguanidine dissolved in 10 ml. of benzene was added to the polymer solution. Agitation was continued for 30 minutes. The mixture, in an 8 ounce screw cap bottle, was a sirupy liquid.

35 The mixing apparatus consisted of 4 clamps attached to a shaft which oscillated in a 90° arc at about 40 cycles per minute in a vertical plane.

40 5.0 g. of monoethyldeca-  
borane was added in the nitrogen atmosphere of a glove box, and mixed on the above shaker for an additional hour.

45 Benzene was removed by vacuum distillation at room temperature, stirring where necessary, for a period of 4 hrs.

50 The residue was heated in a mold cavity at 60° C. for 3 hrs. The fuel was a soft elastic vulcanizate having a gel value of 31 percent. The product was transparent and yellow, and had a few bubbles of gas.

The cured solid was preserved in glass with one atmosphere of nitrogen and was almost unchanged in 6 months time.

Examples XVIII, XIX and XX were performed in a similar manner, as described in Table 5.

TABLE 1

| Example No. | Polybutadiene, g. | Decaborane, g. | Methylcyclohexane, cc. | Reaction Time, Hr. | Reaction Temp., °C. | Pressure, p.s.i.g. | Boron in Prod., Percent |
|-------------|-------------------|----------------|------------------------|--------------------|---------------------|--------------------|-------------------------|
| V-----      | 5.0               | 2.5            | 20                     | 0.5                | 200                 | 40-45              | 16.35                   |
| VI-----     | 5.0               | 5.0            | 20                     | 0.5                | 200                 | 12-35              | 29.73                   |

TABLE 2

| Example No. | Alkylated Decaborane Used     | Alkylated Decaborane Amt., g. | Emulsion Polybutadiene Used, g. | Curing Cond. |            | Cured Fuel   |                |
|-------------|-------------------------------|-------------------------------|---------------------------------|--------------|------------|--------------|----------------|
|             |                               |                               |                                 | Time, Hrs.   | Temp., °C. | Gel, percent | Boron, percent |
| VII-----    | Monoethyldeca-<br>borane----- | 4.7008                        | 1.9981                          | 16           | 55         | 15           | 49.7           |
| VIII-----   | Diethyldeca-<br>borane-----   | 7.3575                        | 1.4899                          | 16           | 33-55      | 2            | 50.0           |
| IX-----     | Triethyldeca-<br>borane-----  | 8.9793                        | 1.5005                          | 24           | 55         | 0.51         | 42.4           |

TABLE 3

| Example No. | Deca. Added, g. | Alk. deca. Used     | Borane-Polybutadiene Mix. Portion, g. | Ratio in Mix., g. |               | Curing Cond. |            | Cured Fuel   |                |
|-------------|-----------------|---------------------|---------------------------------------|-------------------|---------------|--------------|------------|--------------|----------------|
|             |                 |                     |                                       | Borane            | Polybutadiene | Time, Hrs.   | Temp., °C. | Gel, Percent | Boron, Percent |
| X           | 0.0113          | Monoethyldecaborane | 1.1131                                | 4.7008            | 1.9981        | 16           | 55         | 24           | 47.5           |
| XI          | 0.0276          | Diethyldecaborane   | 2.7774                                | 7.3575            | 1.4999        | 16           | 55         | 1            | 49.7           |
| XII         | 0.1921          | Triethyldecaborane  | 6.4224                                | 8.9793            | 1.5005        | 16           | 55         | 0            | 43.2           |

TABLE 4

| Borane                        | Example XIII        | Example XIV       | Example XV         |
|-------------------------------|---------------------|-------------------|--------------------|
|                               | Monoethyldecaborane | Diethyldecaborane | Triethyldecaborane |
| <b>Ingredients:</b>           |                     |                   |                    |
| Borane, g.                    | 1.0694              | 0.9965            | 0.9875             |
| Polybutadiene, g.             | 1.0101              | 1.0002            | 1.0014             |
| Sulfur, g.                    | 0.0205              | 0.0202            | 0.0200             |
| Butyl Eight, g.               | 0.0217              | 0.0184            | 0.0209             |
| Benzene, g.                   | 10.0077             | 10.0070           | 10.0027            |
| Total Fuel, g.                | 2.1217              | 2.0353            | 2.0298             |
| <b>Solvent removed:</b>       |                     |                   |                    |
| Benzene recovery, g.          | 9.2180              | 9.4131            | 9.2935             |
| Fuel recovery, g.             | 2.1288              | 2.0293            | 2.0279             |
| Benzene recovery, percent     | 92.2                | 94.1              | 92.9               |
| Fuel recovery, percent        | 100.3               | 99.7              | 99.9               |
| <b>Extraction:</b>            |                     |                   |                    |
| Benzene, 1st addition, g.     | 57.9566             | 50.7483           | 52.5532            |
| Benzene, 2d addition, g.      | 42.8111             | 43.6021           | 42.7189            |
| Total Benzene, g.             | 100.7677            | 94.3504           | 95.2721            |
| Recovered Benzene, g.         | 97.3290             | 90.1261           | 90.5733            |
| Recovered Benzene, percent    | 96.8                | 95.5              | 95.0               |
| <b>Gel Content:</b>           |                     |                   |                    |
| Weight of Gel, g.             | 1.0350              | 0.8759            | 0.8691             |
| Gel based on Fuel, percent    | 48.7                | 43.0              | 42.8               |
| Gel based on Polymer, percent | 102.4               | 87.6              | 86.9               |
| Boron in Gel, percent         | 2.41, 2.30          | 1.53, 1.08        | 1.11, 1.07         |

TABLE 5

| Mixture                    | Example XVII              | Example XVIII             | Example XIX         | Example XX                               |
|----------------------------|---------------------------|---------------------------|---------------------|------------------------------------------|
| Polybutadiene, g.          | 4.45                      | 3.4                       | 2.35                | 4.05                                     |
| Benzene, ml.               | 50                        | 50                        | 50                  | 50                                       |
| Diphenylguanidine, g.      | 0.0114                    | 0.0085                    | 0.0059              | 0.0101                                   |
| Borane                     | Monoethyldecaborane       | Diethyldecaborane         | Triethyldecaborane  | Crude monoethyl decaborane. <sup>1</sup> |
| Borane, g.                 | 5.0                       | 6.6                       | 7.65                | 5.95                                     |
| Boron, percent calculated  | 40                        | 40                        | 40                  | 40                                       |
| Physical properties        | Soft, elastic vulcanizate | Soft, elastic vulcanizate | Soft, tacky uncured | Soft, elastic vulcanizate                |
| Gel Value, percent         | 31                        | 21                        | 15                  | 33                                       |
| Boron in Gel, percent      | 1.5                       | 1.9                       | 4.8                 | 1.6                                      |
| After storage for 6 months | Almost unchanged          | Almost unchanged          | Almost unchanged    | Almost unchanged                         |

<sup>1</sup> Containing 65.1% monoethyldecaborane, 29.7% diethyldecaborane, 4.0% triethyldecaborane and 1.0% decaborane.

The ethyldecaboranes used in Examples IV and VII to XX were obtained from a Friedel-Crafts reaction of decaborane-14 ( $B_{10}H_{14}$ ) and an ethyl halide, in the presence of a ferric chloride catalyst. The product of this reaction consisted of a mixture of ethyldecaborane, diethyldecaborane and triethyldecaborane. These constituents were separated by a fractional distillation at reduced pressures. At a pressure of about 0.2 mm. of mercury, monoethyldecaborane boils at approximately 30° C., diethyldecaborane at 45° C. and triethyldecaborane at 65° C. By this method of separation products were obtained having a purity of greater than 99 percent.

The boron containing solid materials produced by practicing the method of this invention can be employed as ingredients of solid propellant compositions in accordance with general procedures which are well understood in the art, since the solid materials are readily oxidized using conventional solid oxidizers, such as ammonium perchlorate, potassium perchlorate, sodium perchlorate, aluminum perchlorate, lithium perchlorate, ammonium nitrate and the like. In formulating a solid propellant composition employing one of the materials produced in accordance with the practice of this invention, generally from 10 to 35 parts by weight of the boron-containing material of this invention and from 65 to 90 parts by

weight of oxidizer such as ammonium perchlorate are present in the final propellant composition.

The polybutadiene-borane reaction product can be subdivided by means of conventional equipment designed to reduce the size of resilient materials, e.g., such devices which cut, chop or tear the feed material into a divided product as the well-known rotary knife cutters and granulators. The oxidizer can be reduced in size by conventional equipment, e.g., a hammer mill. In formulating a propellant the finely divided reaction product and oxidizer can then be intimately admixed in conventional mixing equipment employing rotating blades, e.g., kneaders or Baker-Perkins mixers, along with a binder such as an additional quantity of polybutadiene, or other rubber and curing agents. This resulting intimate admixture can then be cast or pressed into the desired form and cured.

Propellant compositions can also be prepared by intimately admixing the polybutadiene, the borane, the oxidizer and other conventional curing agents if desired and curing this resulting intimate admixture.

In addition to the oxidizer and oxidizable material, the final propellant can contain another binder as previously stated. A binder of an artificial resin type, such as phenol-formaldehyde, is useful. The function of this resin is to give the propellant mechanical strength and at the

same time improve its burning characteristics. In manufacturing a suitable propellant using a binder, the solid reaction product mixed with the proper proportions of finely divided oxidizer is admixed with a high solids content solution of a partially condensed phenol-formaldehyde resin, the proportion being such that the amount of the resin is about from 5 to 10 percent by weight, based upon the weight of the oxidizer and the boron material. The ingredients are thoroughly mixed with the simultaneous removal of the solvent, e.g., by use of a vacuum, and following this the solvent-free mixture is molded into the desired shape as by extrusion. Thereafter, the resin in the mixture can be cured, e.g., by heating at moderate temperatures, e.g., 50-200° C. Conventional and suitable methods of formulation of solid propellant compositions are further described in U.S. Patent 2,622,277 of Bonnell and U.S. Patent 2,646,596 of Thomas.

The following examples illustrate the formulation of solid propellant compositions utilizing the solid boron-containing reaction product of this invention which has been prepared without incorporation of oxidizer.

*Example XXI*

20 pounds of the solid boron-containing material of Example II (mean particle size 840 microns) and 80 pounds of ammonium perchlorate oxidizer (mean particle size 840 microns) are introduced into a Baker-Perkins mixer along with 10 pounds of a solution of a phenol formaldehyde resin in toluene and the three components intimately admixed with the simultaneous removal of the solvent by means of a vacuum. The resulting solvent-free homogeneous solid is molded or extruded and cut into cylindrical grains of about 2 inches in diameter and 3 inches in length. The grains are then heated in an oven to about 100° for the necessary time to cure the resin in the grains. The resulting grains are an intimate admixture of solid fuel and oxidizer with resin binder.

The product of this invention can be utilized in its extracted form, that is, after the uncombined decaborane or lower alkyl decaborane has been removed from the final reaction product by extraction with a suitable solvent. The unextracted reaction product, however, can also be advantageously used as a propellant. The unextracted product contains a quantity of decaborane or lower alkyl decaborane homogeneously dispersed throughout. When combined with an oxidizer in the manner previously described and ignited, both the combined product and the decaborane or lower alkyl decaborane burn readily. The unextracted product has the advantage of containing a higher percentage of boron (an element having a high heat of combustion) homogeneously dispersed in a form which can be easily admixed with a suitable oxidizing agent and which will burn liberating a larger quantity of energy than the extracted product.

What is claimed is:

1. A solid high energy fuel composition consisting essentially of the product of reaction of polybutadiene rubber and a borane selected from the group consisting of decaborane and lower alkyl decaboranes and mixtures thereof at a temperature of about 20 to 300° C. and in amounts of about 0.05 to 10 parts by weight of borane per part of polybutadiene rubber.
2. The composition of claim 1 in which the borane is decaborane.
3. The composition of claim 1 in which the borane is diethyldecaborane.
4. The composition of claim 1 in which the borane is monoethyldecaborane.

5. The composition of claim 1 in which the borane is triethyldecaborane.

6. The composition of claim 1 in which the polybutadiene and borane are reacted in an amount of about 0.5 to 3.5 parts of borane per part of polybutadiene.

7. The composition of claim 6 in which the borane is decaborane.

8. The composition of claim 6 in which the borane is diethyldecaborane.

9. The composition of claim 6 in which the borane is monoethyldecaborane.

10. The composition of claim 6 in which the borane is triethyldecaborane.

15 11. The method of preparing a solid high energy fuel composition which comprises reacting polybutadiene rubber with a borane selected from the group consisting of decaborane and lower alkyl decaboranes and mixtures thereof at a temperature of about 20 to 300° C. and in amounts of about 0.05 to 10 parts by weight of borane per part of polybutadiene rubber.

12. The method of claim 11 in which the borane is decaborane.

13. The method of claim 11 in which the borane is diethyldecaborane.

25 14. The method of claim 11 in which the borane is monoethyldecaborane.

15 15. The method of claim 11 in which the borane is triethyldecaborane.

16. The method of claim 11 in which the polybutadiene 30 and borane are reacted in amounts of 0.5 to 3.5 parts of borane per part of polybutadiene.

17. The method of claim 16 in which the borane is decaborane.

35 18. The method of claim 16 in which the borane is diethyldecaborane.

19. The method of claim 16 in which the borane is monoethyldecaborane.

20. The method of claim 16 in which the borane is triethyldecaborane.

40 21. A solid high energy fuel composition consisting essentially of the product obtained by reacting at a temperature of 80 to 140° C. equal proportions of polybutadiene and decaborane.

45 References Cited by the Examiner

UNITED STATES PATENTS

2,558,559 6/1951 Hurd et al.

2,791,883 5/1957 Moore et al.

50 OTHER REFERENCES

Hurd, "Chemistry of the Hydrides," New York, John Wiley & Sons, Inc., 1952, page 94.

Arendale, Industrial and Eng. Chem., April 1956, pp. 725-6.

55 Ley, Coast Artillery Journal, Jan.-Feb. 1948, p. 27.

Ritchey, Chem. and Eng. News, Nov. 11, 1957, pp. 78-82.

Major, Chem. Eng. Progress, vol. 54, No. 3, March 1958, pp. 49-54.

60 Proell et al., The J. of Space Flight, vol. 2, No. 1, January 1950, pp. 1-9.

Chem. and Eng. News, May 27, 1957, pp. 18-23.

"Jet Propulsion," Air Technical Service Command (1946), p. 158.

65 BENJAMIN R. PADGETT, *Acting Primary Examiner*,

LEON D. ROSDOL, ROGER L. CAMPBELL,

Examiners.

UNITED STATES PATENT OFFICE  
CERTIFICATE OF CORRECTION

Patent No. 3,266,958

August 16, 1966

Jack D. Breazeale et al.

It is hereby certified that error appears in the above numbered patent requiring correction and that the said Letters Patent should read as corrected below.

Column 2, line 22, for "32.5" read -- 325 --; column 4, line 28, for "3.7" read -- 33.7 --.

Signed and sealed this 1st day of August 1967.

(SEAL)

Attest:

EDWARD M. FLETCHER, JR.

Attesting Officer

EDWARD J. BRENNER

Commissioner of Patents